

Nov. 20, 1923.

1,474,596

F. W. KENT

PHOTOGRAPHIC TRANSFER PAPER AND PROCESS OF MAKING SAME

Filed Feb. 8, 1921



Invantor  
Frank W. Kent  
By Cushman, Bryant & Co. only  
attn: [unclear]

## UNITED STATES PATENT OFFICE.

FRANK WILLIAM KENT, OF STREATHAM HILL, LONDON, ENGLAND.

## PHOTOGRAPHIC TRANSFER PAPER AND PROCESS OF MAKING SAME.

Application filed February 8, 1921. Serial No. 443,412.

*To all whom it may concern:*

Be it known that I, FRANK WILLIAM KENT, a subject of the King of Great Britain, residing at 5 Thornton Avenue, Streatham Hill, in the county of London, England, have invented certain new and useful Improvements in or Relating to Photographic Transfer Paper and Processes of Making Same, of which the following is a specification.

This invention relates to photographic transfer processes in which the film of photographic emulsion after being exposed, developed, fixed and washed to form a positive picture is transferred from its original base or support to a mount of wood, paper, glass, porcelain, metal or other suitable material, by means of a suitable adhesive, for example a 5 per cent solution of warm gelatine, in the usual and known manner, the base after drying being then stripped off. In the manufacture of the printing materials intended to be employed in the above process the base is composed of paper which has been passed through a bath of paraffin wax and dried, and a substratum has been applied to this base to enable the emulsion to be applied evenly to the said base in the first instance, to prevent the emulsion from stripping off the base during the subsequent operations of developing, fixing, washing or toning, and afterwards to allow the gelatine emulsion to be stripped from its original base when required. This substratum has in certain cases consisted of a waterproof resinous material such as sandarac or mastic. This, however, being insoluble in water, portions of it were liable to remain adhering to the emulsion in the finished picture and to spoil the effect of the same.

According to this invention the substratum is produced by a solution containing as its chief ingredient an emulsion hardening agent, such as is employed, for example, as a component of the ordinary bromide emulsion. A suitable hardening agent is chrome alum or formaldehyde but ordinary alum may be used. The hardening agent also serves to bind the emulsion to the substratum, and therefore in that sense may also be regarded as a binding agent. An anti-greasing agent such as quillaia bark is also added to allow of even spreading of the emulsion on the substratum and some glycerine is also preferably added. The improved substratum can be used with various

emulsions containing gelatine and is not restricted to use with a bromide emulsion. The emulsion employed should be of a tough nature.

In the accompanying drawing is shown on an enlarged scale a section of a portion of a transfer film on a base such as paper. Between the film and the base is interposed the substratum. In the said drawing, A, indicates the base and B the film or emulsion, while the substratum on which the film emulsion is laid, is shown at C.

I preferably employ a plain photographic base (that is, a paper which has no baryta coating) impregnated with paraffin wax in a known manner, that is, by passing it through a bath of paraffin wax at a low degree of saturation, for example, ten grains of paraffin wax dissolved in one oz. of benzol or other suitable solvent is a suitable strength although a weaker or stronger solution might be used if desirable.

This waxed paper when dried is coated on one side only with a substratum which may be composed as follows:—

1 oz. water.  
4 drachms of 5 per cent solution of chrome alum.  
1 oz. alcohol or methylated spirit.  
4 dr. of 2 per cent solution of quillaia bark.  
½ dr. glycerine.

The respective proportions may be varied to suit climatic or other conditions.

For example, if the paper is chilled immediately after coating with the emulsion the solution is made with a greater strength of chrome alum or other hardening agent and quillaia bark or other anti-greasing agent. The formaldehyde or other hardening agent which may be used instead of chrome alum is employed in a suitable strength to give a corresponding hardening effect. Or any suitable mixture of hardening agents may be employed.

The alcohol may be omitted, but in that case the substratum will take a much longer time to dry.

The chrome alum is employed not only for its hardening and binding effect, but also as a preventative against frilling and blistering, the quillaia bark to enable a smooth and even flow of the solution over the surface of the waxed paper, and the glycerine to give flexibility and to bind the other ingredients. The substratum is applied to the

waxed base in the usual manner and in leaving the bath the base may if found desirable be subjected to the action of one or more scrapers or "doctors" in order to reduce the quantity of the substratum carried by the base, and such scrapers might in certain cases be also used when waxing the paper.

An ordinary photographic gelatine emulsion is then applied over this substratum when dry, in the usual manner, and a positive print taken which can be developed and toned by any standard formula whilst still on the waxed base.

15 In the preparation of the substratum intended for transferring photographs on to woven fabrics, the previous formula should be altered to the following, which may also be varied to suit circumstances.

20 Water, 1 oz.  
Chrome alum, 2 dr. of 5 per cent solution.  
Alcohol, 1 oz.  
Quillaia bark, 1 dr. of 2 per cent solution.  
Glycerine, 1 dr.

25 After developing, fixing and washing the print in this process, a warm 5 per cent gelatine solution is brushed over the face side of the wet print which is to be ironed into the fabric. The print is laid on the fabric 30 and dry cloths or fluffless blotting paper placed under the fabric and over the print, and an iron heated to 150 to 200 degrees Fahrenheit is repeatedly passed over the cloths or blotting paper, with occasional inversion, until the print is dried. The wax 35 paper can then be stripped off in the ordinary way. The fabric with the picture thereon can be afterwards placed in a bath of 2% formaldehyde solution (which may also contain glycerine) for about three minutes at atmospheric temperature, and dried with a hot iron or otherwise, the iron being only required to remove creases. The fabric is then washable by ordinary domestic processes without affecting the photograph.

45 The components of the solution used for this substratum, being of the same nature as those which are employed in the emulsion itself, will not injuriously affect the emulsion.

50 A quantity of the base coated with this substratum can be re-reeled, packed, and sent away to be afterwards coated with any desired emulsion, which is difficult in the 55 case where resinous and other known substratum are employed.

An important advantage arising from the use of this solution is the effect of the chrome alum or other hardening agent in 60 binding the constituents of the substratum or some portion of them, to the gelatine emulsion, so that although soluble in water a sufficient portion of the substratum remains, and after removing the waxed base 65 will remain smooth and transparent, and

thus will not give any powdery or other detrimental effect on the finished print, being in fact imperceptible. The action of the hardening and binding agent forming the most important part of the substratum 70 upon the adjacent emulsion is one of the chief characteristics of the new substratum as compared with those hitherto employed and enables a much more satisfactory transfer of the print to be obtained and enhances 75 its effect.

What I claim and desire to secure by Letters Patent of the United States is:—

1. A process for preparing a photographic transfer film, which consists in applying to a suitable base a substratum comprising as its main ingredient an emulsion hardening agent in active condition and in coating the said substratum when in its dry condition with a sensitive emulsion. 80

2. A process for preparing a photographic transfer film, which consists in applying to a suitable base a substratum solution free from gelatin comprising as its main ingredient chrome alum drying the 90 said substratum and in coating the dried substratum with a sensitive emulsion.

3. A process for preparing a photographic transfer film, which consists in applying to a suitable base a substratum comprising emulsion hardening and anti-greasing agents and in coating the said substratum when in a dry condition with a sensitive emulsion. 95

4. A process for preparing a photographic transfer film, which consists in applying to a suitable base a substratum comprising emulsion hardening and anti-greasing agents and a small proportion of glycerine and in coating the said substratum 100 with a sensitive emulsion. 105

5. A process for preparing a photographic transfer film, which consists in applying to a suitable base a substratum comprising an emulsion hardening agent and a 110 small proportion of quillaia bark and in coating the said substratum with a sensitive emulsion.

6. A process for preparing a photographic transfer film, which consists in coating a waxed paper base with a substratum comprising as its main ingredient an emulsion hardening agent and in coating the said substratum with a sensitive emulsion. 115

7. A process for preparing a photographic transfer film, which consists in treating a waxed paper base with a solution of chrome alum, quillaia bark and glycerine to form when dry a substratum upon the 120 said base and in coating the substratum with a sensitive emulsion.

8. A photographic transfer paper comprising a waxed paper base coated with a substratum containing as its main ingredient an emulsion hardening agent in active 130

condition, and a sensitive emulsion upon the said substratum.

9. A photographic transfer paper comprising a waxed paper base, a substratum containing an emulsion hardening agent and an anti-greasing substance and a sensitive emulsion upon the said substratum.

10. A photographic transfer paper comprising a waxed paper base and a substratum consisting of chrome alum, quillaia bark and a small proportion of glycerine and a sensitive emulsion upon the said substratum. 10

FRANK WILLIAM KENT.